

## UNITED STATES PATENT OFFICE

2,312,208

## COMPOUNDED HYDROCARBON OIL

James O. Clayton and Bruce B. Farrington, Berkeley, Calif., assignors to Standard Oil Company of California, San Francisco, Calif., a corporation of Delaware

No Drawing. Application April 12, 1941,  
Serial No. 388,299

25 Claims. (Cl. 252—34)

This invention relates to a new and useful composition of matter comprising a hydrocarbon oil and a salt of organic substituted acids of boron. More particularly, the invention involves compounded oils containing an oxide, sulfide or selenide in which an oxygen, sulfur or selenium atom is directly attached to a metal and a boron atom.

The present invention involves the discovery that dispersion in hydrocarbon oils of certain oxides, sulfides or selenides containing the group—

(A) (X) (B) (R)

in which A represents a salt-forming element or radical, X is oxygen, sulfur or selenium, B is boron, and R is an organic radical, imparts new, unpredictable and desirable properties to the composition. These new properties render the compounded oil particularly useful for various purposes. Increased resistance to deterioration under oxidizing conditions comprises one of the principal advantages of the compounded oils of this invention, but it is to be understood that the invention is not limited to this feature. Different compounds of the general type herein involved vary in their degree of effectiveness and may impart one or more other desirable properties to the composition. For example, certain of the compounds may reduce the amount of wear produced in lubrication of metal surfaces as compared with wear resulting with a straight uncompounded lubricating oil. The same or other compounds inhibit corrosion of alloy bearings of the type represented by copper-lead or cadmium-silver bearing metals. In general, however, it has been discovered that the new compositions herein disclosed are more stable to deterioration by heat and oxidation than is a hydrocarbon oil with which the compositions are compounded. The new compounds of this invention are therefore useful where a stabilized oil is desired and resistance to deterioration is important. An example of such utility is their use as lubricating oils, particularly in internal combustion engines, to inhibit gumming of pistons, sticking of piston rings, sludge formation in the crankcase, and the like. The compositions are also useful as heat transfer fluids where it may be desirable to inhibit or prevent the formation of a deposit on the metal surfaces from or to which heat is being conveyed. Likewise, the increased resistance to oxidation imparted to the oils by the compounds of this invention finds various applications in an insulating, switch or transformer oil.

Compounds of the type herein involved and containing the group—

(A) (X) (B) (R)

as previously identified, may be regarded as salts of substituted acids of boron. Metal salts of substituted oxyacids of trivalent boron are preferred compounding agents. Metals preferred as components of the salts utilized in this invention are metals selected from groups II, III, IV and VI of Mendeleeff's Periodic Table of the Elements. Specific examples of such metals are: calcium, strontium, barium, magnesium, zinc, cadmium, aluminum, zirconium, bismuth, tin, lead, chromium and molybdenum. Salts of iron, cobalt, nickel, manganese, vanadium, sodium, potassium, copper and silver comprise additional examples of metals falling within the broader aspects of the invention. Salt-forming radicals such as the ammonium and amine radicals are not precluded.

The compounds of this invention are preferably formed from substituted oxyacids of trivalent boron of the following formulae:



25 organic boronic acids;



30 organic boronic acids;



35 monoesters of orthoboric acid;



40 diesters of orthoboric acid;

45 where R and R' are radicals of hydrocarbon structure. It is understood that we do not preclude R and R' having substituents, such as the polar radicals OH, SH, Cl, NH<sub>2</sub> and COOH. Likewise, by the term "radicals of hydrocarbon structure" it is intended to include radicals containing ether, sulfide and ester groups. Examples of preferred type acids are alkyl or alkaryl boronic acids having at least twelve carbon atoms in the molecule. However, it is to be understood that the broader aspects of the invention include the use of deriva-

tives of other types of organic substituted acids of boron.

Additional examples of organic substituted acids of boron which may be used in forming the salts of the present invention are as follows:



organic monothio-boronic acids;



organic dithio-boronic acids;



organic thio-borinic acids;



monoesters of monothio-organo boric acid;



monoesters of organo monothio-boronic acid;



monoesters of organo dithio-boronic acid;



diesters of monothio-organo boric acid;



diesters of thio-organo thio-boronic acid;



diesters of dithio-organo boric acid;



diesters of dithio-organo thio-boronic acid.

In all of the foregoing formulae R and R' are radicals of hydrocarbon structure. Throughout the specification and claims the term "radical of hydrocarbon structure" includes:

(a) Alkyl radicals, such as amyl, isoamyl, hexyl, heptyl, octyl, the isomeric octyls, lauryl,

dodecyl (normal or branched chain), tetradecyl and cetyl (normal or branched chain) radicals;

(b) Aryl, such as the phenyl, diphenyl and naphthyl, radicals;

(c) Aralkyl, such as phenyloctadecyl and similar alkyl radicals connected to the boron atom and having an aryl group as a substituent in the alkyl chain;

(d) Alkaryl, such as methylphenyl, cetyl-phenyl, and other radicals where the aryl group is directly attached to the boron atom and is substituted with an alkyl group;

(e) Cyclic nonbenzenoid radicals, such as cyclohexyl or other alicyclic radicals;

(f) Oxy radicals such as those in which the hydrogen of an hydroxyl group has been replaced by esterification, etherification, neutralization with a metal, or the like;

(g) Radicals containing thio, amino, halogen or other groups.

It should be borne in mind that in the previously listed type formulae all of the acids listed may not exist as such and that it is the salt-like derivatives thereof with which the present invention is concerned. Accordingly, existence of the free acid in a stable form is not a prerequisite to the preparation of the derivatives thereof contemplated herein.

In general, salts and preferably polyvalent metal salts of organic substituted derivatives of acids of boron, such as orthoboric,  $\text{H}_3\text{BO}_3$ ; mesoboric,  $\text{H}_4\text{B}_2\text{O}_5$ ; metaboric,  $\text{H}_2\text{B}_2\text{O}_4$ ; dihydrodi-boric,  $\text{H}_4\text{B}_2\text{O}_8$ ; hexahydrotetraboric,  $\text{H}_6\text{B}_4\text{O}_9$  (once called pyroboric acid); dihydrotetraboric,  $\text{H}_2\text{B}_4\text{O}_7$ ; hexahydrohexaboric,  $\text{H}_6\text{B}_6\text{O}_{12}$ ; dihydrohexaboric,  $\text{H}_2\text{B}_6\text{O}_{10}$ ; hexahydro-octoboric,  $\text{H}_8\text{B}_8\text{O}_{15}$ ; dihydro-octoboric,  $\text{H}_2\text{B}_{10}\text{O}_{13}$ ; dihydro-decaboric,  $\text{H}_2\text{B}_{10}\text{O}_{16}$ ; and dihydrononadecaboric,  $\text{H}_2\text{B}_{12}\text{O}_{19}$ ; fall within the broadest aspects of the invention. By "substituted" or "substituted derivatives of" acids of boron whenever used herein it is intended to designate acids containing an organic group of the type previously listed, which acids may be either an oxy and thio or a mixed oxy and thio acid of boron. The organic groups may be either directly attached to the boron atom of the compound or attached thereto through an intervening atom, such as oxygen or sulfur. The term "oxyacid of boron" is intended to designate acids in which at least one oxygen atom intervenes between the hydrogen and boron atom of the parent acid.

The preferred acids are substituted acids of trivalent boron and the preferred salts comprise the magnesium, aluminum, calcium, barium, tin, and chromium salts of these acids. Examples of such salts are: magnesium, aluminum, calcium, barium, tin and chromium monododecyl, mono-tetradecyl, monocetyl, mono-octadecyl, mono-(amylphenyl), mono-decylphenyl, mono-(dodecylphenyl), mono-(tetradecylphenyl), mono-(cetylphenyl), mononaphthyl, dihexyl, dioctyl, didecyl, didodecyl, ditetradecyl, dicetyl, dioctadecyl, diphenyl, dibenzyl, di-(ethylphenyl), di-(amylphenyl), di-(decylphenyl), di-(dodecylphenyl), di-(cetylphenyl) and di-(cyclohexyl), borates; magnesium, aluminum, calcium, barium, tin and chromium dodecyl, tetradecyl, cetyl, octadecyl, amylphenyl, decylphenyl, dodecylphenyl, tetradecylphenyl, cetylphenyl and naphthyl, boronates; and magnesium, aluminum, calcium, barium, tin and chromium dihexyl, dioctyl, didecyl, didodecyl, ditetradecyl, dicetyl, dioctadecyl, diphenyl, dibenzyl, di-(ethylphenyl), di-(amylphenyl), di-(decylphenyl).

phenyl), di-(dodecylphenyl) and di-(cetyl-phenyl), borinates.

The substituted acids of boron utilized in the preparation of the salts of this invention may be obtained by known methods. For example, the monoesters of boric acid and diesters of boric acid are obtainable by hydrolysis of the triester, and the desired salts may be prepared from either the unneutralized partially hydrolyzed ester or from the sodium salt thereof by reaction with the desired metal ion.

The diesters of boronic acids are obtainable, for example, by the slow oxidation of trialkyl borine. Also, the aliphatic and aromatic boronic acids can be prepared readily by the reaction of Grignard reagents upon alkyl esters of boric acid or the etherate of boron trifluoride instead of an alkyl borate.

In general, it may be explained that boric esters may be prepared by the action of alcohols on boric anhydride under pressure. These esters react with Grignard's reagents to form the boronic acids according to the equation:



When magnesium phenyl bromide is utilized, a methylating action occurs so that, in addition to phenyl boronic acid, toluene is obtained. The lower boronic acid esters are readily hydrolyzed by cold water to yield the free boronic acid.

The following will illustrate in more detail a method of preparing a typical substituted acid of boron. Alkyl boronic acids in general may be prepared by this procedure without essential modification:

A 1-liter 3-necked flask is fitted with an efficient mercury sealed stirrer and one neck provided with a low temperature thermometer and a glass tube for the introduction of nitrogen. The remaining neck carries a 500 cc. separatory funnel and an outlet tube for nitrogen or other inert gas. The nitrogen outlet tube and the top of the separatory funnel are connected to two arms of a Y-tube, the third arm of which is sealed by a mercury valve. Dry nitrogen, purified over sulfuric acid and alkaline pyrogallol, is allowed to flow through the apparatus for about twenty minutes. Then 55 grams (0.53 mol) of pure methyl borate is added quickly through the separatory funnel and washed through with 150 cc. of anhydrous ether. The flask is suspended in a Dewar dish containing a mixture of acetone and solid carbondioxide and the solution stirred during cooling. When the internal temperature has fallen to about  $-75^{\circ}$ , 300 cc. (0.5 mol) of alkyl magnesium bromide solution (1.66 N) is introduced slowly through the separatory funnel over a period of several hours. The flow of nitrogen and vigorous stirring are maintained during the addition and the temperature held below  $-70^{\circ}$ . During the addition a voluminous precipitate separates. When the addition is complete, the mixture is stirred at  $-70^{\circ}$  for several hours and allowed to stand in the cooling bath over night to insure completion of the reaction. The flask is then opened momentarily and the cake of precipitate broken into small amounts. The apparatus is reassembled and 300 cc. of water containing 30 cc. of sulfuric acid added with stirring and cooling. The ethereal layer is separated and the aqueous layer extracted with 50 cc. of ether. The extract is combined with the main ether layer. The ethereal solution is concentrated on a steam bath and distillation continued until all material volatile at the temperature of the bath

is removed. The acid which separates upon cooling the residual liquid is filtered with suction and may be dried in a nitrogen-filled desiccator over 65% sulfuric acid. This crude acid may be purified by warming with 275 cc. of toluene, the solution filtered at  $60^{\circ}$  C. and chilled thoroughly to cause crystallization.

The necessity for maintaining extremely low temperatures, as in the above method, may be avoided by using a less volatile ester as a starting material, for example, by using n-butyl borate.

*Example 1.*—n-Tetradecanol is converted to the bromide (B. P. 132-135° F. at 2 mm.). The Grignard reagent from this bromide is added to n-butyl borate and gives a crude impure acid contaminated with the hydrocarbon  $C_{28}H_{58}$ . The latter may be removed by dissolving the crude acid in 95% alcohol and chilling. The purified n-tetradecane boronic acid is obtained by evaporation of the alcohol and crystallization from petroleum ether.

*Example 2.*—Cetyl alcohol is converted to the bromide. The Grignard reagent from this bromide is added to a suitable borate ester such as the n-butyl borate.

*Example 3.*—Phenyl magnesium bromide is added to n-butyl borate to obtain the benzene boronic acid as in the foregoing examples.

*Example 4.*—Cetylphenyl magnesium bromide obtained from cetyl benzene may be used to prepare cetylphenyl or cetyl benzene boronic acid.

As previously indicated, salts of the foregoing acids may be prepared by treating the acid with aqueous alcoholic sodium hydroxide and then precipitating the various salts by adding an aqueous solution containing the desired metal ion. For example, cetyl boronic acid is reacted with aqueous alcoholic sodium hydroxide to give sodium cetyl boronate from which various salts are prepared as follows:

*Example 5.*—Aqueous calcium chloride is added to the aqueous alcoholic solution of sodium cetyl boronate to precipitate calcium cetyl boronate. The precipitate is filtered, washed and dried, or it may be taken up immediately upon precipitation by dissolving in an organic solvent such as a hydrocarbon mineral oil.

*Example 6.*—To prepare the zinc salt, aqueous zinc chloride solution is added to the alcoholic sodium cetyl boronate solution.

*Example 7.*—To prepare the magnesium salt, aqueous magnesium chloride or magnesium sulfate solution is added to the alcoholic sodium cetyl boronate solution.

*Example 8.*—To prepare the aluminum salt, aqueous aluminum chloride or aluminum sulfate solution is added to the alcoholic sodium cetyl boronate solution.

*Example 9.*—To prepare the tin salt, aqueous tin chloride solution is added to the alcoholic sodium cetyl boronate solution.

*Example 10.*—To prepare the lead salt, aqueous lead acetate solution is added to the alcoholic sodium cetyl boronate solution.

*Example 11.*—To prepare the chromium salt, aqueous chromic sulfate or chrome alum solution is added to the alcoholic sodium cetyl boronate solution.

*Example 12.*—To prepare the manganese salt, aqueous manganese sulfate solution is added to the alcoholic sodium cetyl boronate solution.

*Example 13.*—To prepare the nickel salt, aqueous nickel chloride solution is added to the alcoholic sodium cetyl boronate solution.

*Example 14.*—To prepare the cobalt salt, aque-

ous cobalt chloride solution is added to the alcoholic sodium cetyl boronate solution.

A borinic acid is obtained when boron diphenyl chloride or bromide is treated with sodium hydroxide and the clear solution neutralized with hydrochloric acid. The dibenzene borinic acid results and readily forms alkali metal salts which in turn may be converted to a polyvalent metal salt by reaction with the desired metal ion.

Salts of the partially esterified boric acids may be prepared by partially hydrolyzing the ester with sodium hydroxide to obtain the sodium salt of the partial ester. Other salts may be precipitated by double decomposition in accordance with the methods described in the foregoing examples.

Among the benefits which may be derived from the incorporation of the compounds of this invention in lubricating oils are inhibition of corrosion of bearing metals and increased stability of the oil as indicated by lower neutralization number and lower A. S. T. M. naphtha insolubles after use. Table I gives data illustrating these properties.

In the tests whose results are summarized in Table I, thin sheets of the indicated bearing metals were cut into strips (copper-lead,  $\frac{1}{8}'' \times 1\frac{3}{4}'' \times \frac{3}{32}''$ ), and these strips were immersed in the exemplified oils carried in  $2'' \times 20''$  glass test tubes; these test tubes were carried in an oil bath maintained at  $300^{\circ}\text{F.} \pm 1^{\circ}\text{F.}$  Each test tube contained approximately 300 cc. of oil, and air was bubbled through each tube at the rate of 10 liters per hour. At the end of each of three 24-hour periods, the strips were removed from the oils, washed with petroleum ether and carefully wiped with a soft cotton cloth; weight losses of the strips were measured in connection with the weight of each individual strip. The duration of the tests was 72 hours.

Table I

| Oil                                                                        | Weight loss in mg.<br>copper-lead |             |             | Inspections,<br>72 hours                |                                                   |
|----------------------------------------------------------------------------|-----------------------------------|-------------|-------------|-----------------------------------------|---------------------------------------------------|
|                                                                            | 24<br>hours                       | 48<br>hours | 72<br>hours | Neutral-<br>iza-<br>tion<br>num-<br>ber | A. S.<br>T. M.<br>naph-<br>tha<br>insol-<br>ubles |
| Acid refined S. A. E. 30 naphthenic base oil                               | 1.0                               | 5.7         | 35.2        | 4.07                                    | 114                                               |
| Acid refined S. A. E. 30 naphthenic base oil + 0.5% calcium cetyl boronate | 1.8                               | 2.6         | 2.8         | 1.40                                    | 50                                                |

Among the beneficial effects which flow from the incorporation of the above-described compounds in a hydrocarbon oil of the lubricating oil class is the prevention of piston ring sticking, or its marked postponement, under very severe motor conditions, as for example in Diesel engine or in aircraft spark or compression ignition engine operations.

Table II

| Oil                                                                         | Hours to<br>stick rings | Piston dis-<br>coloration<br>number |
|-----------------------------------------------------------------------------|-------------------------|-------------------------------------|
| Acid refined S. A. E. 30 naphthenic base oil                                | 45                      | Poor.                               |
| Acid refined S. A. E. 30-naphthenic base oil + 0.35% calcium cetyl boronate | >60                     | Improved.                           |

In the tests whose results are summarized in Table II, a single cylinder Lauson gasoline spark-

ignition engine,  $2\frac{3}{8}''$  bore and  $2\frac{1}{2}''$  stroke, loaded with fan dynamometers, was operated under extremely severe conditions, designed to develop fully the tendency of the crankcase lubricant to deteriorate with gum formation and piston ring sticking: operation was at 1600 R. P. M.; engine jacket temperature was maintained at  $375^{\circ}\text{F.}$ ; crankcase oil temperature was maintained at  $220^{\circ}\text{F.}$ ; at periods of fifteen hours the operations were interrupted and the condition of the piston rings determined.

Additional examples of acids of boron, the salts of which are contemplated as addition agents for hydrocarbon oils within the broadest aspects of the invention, are as follows: p-chlorophenyl boronic acid, p-bromophenyl boronic acid, o-anisyl boronic acid, o-phenetyl boronic acid, and o-xylyl boronic acid. The calcium, strontium, barium, magnesium, zinc, cadmium, aluminum, zirconium, bismuth, tin, lead, chromium, molybdenum, iron, cobalt, nickel, manganese, vanadium, sodium, potassium, copper and silver salts of these acids may be utilized.

Reference has previously been made to the fact that amine salts of the acids disclosed in the specification fall within the broader aspects of the invention. Examples of suitable amines are the alkyl amines, such as triethyl amine; the alkylol amines, like triethanolamine; and the aromatic amines, such as aniline. Nitrogen bases obtained from petroleum, and especially reduced nitrogen bases such as homologues of piperidine, are also included as an amine with which the salts of this invention may be made.

The proportion of the addition agents herein disclosed which may be added to hydrocarbon oils according to the principles of the present invention may vary widely, depending upon the uses involved and the properties desired. As little as 0.05% by weight of various of the compounds gives measurable improvements. From approximately 0.1% to 2% of the compounds may be added to lubricants where enhanced stability under oxidizing conditions is desired. More than 2% of the compounds may be utilized for various purposes, e. g. for preparing lubricating greases and concentrates capable of dilution with mineral lubricating oils and the like. Concentrates containing high percentages of the addition agents comprise a convenient method of handling the ingredients and may be marketed as such as addition agents for lubricants in general as well as for other purposes.

The compounded hydrocarbon oils herein disclosed may have one or more advantages depending upon the particular compounding agents selected, the proportions utilized and the environment or use which the compounded oil is to encounter. It should be observed, for example, that even though a compounded oil may be somewhat corrosive to copper-lead or cadmium-silver bearing metals, Babbitt bearings may be little if at all affected by such corrosive action. Hence, compounded oils which may not be particularly desirable for lubrication of copper-lead or cadmium-silver bearings at high temperatures where corrosion becomes a factor of importance may be highly useful and extremely advantageous in conjunction with operations where bearings of Babbitt or other corrosive-resistant bearing metals are utilized. Likewise, compounded oils in which the addition agent is not sufficiently powerful to stabilize the oil against deterioration by oxidation under the most severe conditions may be highly useful in

those applications where the temperatures or oxidizing conditions encountered are not so severe, e. g. in a transformer oil. The present invention in its broader aspects is therefore not limited to the particular ingredients having all or the greatest number of advantages obtainable, but embraces various of the less advantageous addition agents which will find utility in particular applications where all the possible improvements in the properties may not be required or where the standard of performance may not be so high.

In the preparation of either the finished oils of the invention or the bases or concentrates referred to, complete or clear and homogeneous solution is not always necessary. Blending agents or homogenizers may be employed, if desirable, to prevent sedimentation of the less oil-soluble agents but it has been found that the possible detrimental effect of the presence of filterable insoluble materials of this character, if present, is determined largely by the particular conditions attending the contemplated use and that with those addition agents of limited oil-solubility the presence of additional oil-insoluble agents is not in all cases deleterious to the function of the compositions in their intended manner.

The preferred hydrocarbon oil is a mineral lubricating oil fraction such as a moderately acid refined naphthenic base lubricating oil. Other base oil stocks for the compounded oils involved herein may be utilized, e. g. paraffinic oil stocks or highly refined naphthenic oils, as well as synthetic hydrocarbon oils. It is to be understood that the broader aspects of the invention are not limited to any particular base stock since the advantages herein disclosed may be obtained, at least to some degree, with various oils, the selection of which will be determined by conditions and service which the product is to encounter.

The addition agents of this invention may be utilized in hydrocarbon oils containing other compounding agents, such as pour point depressants, oiliness agents, extreme pressure addition agents, blooming agents, compounds for enhancing the viscosity index of the hydrocarbon oil, and auxiliary stabilizing agents such as metal alcoholates, metal salts of phenols containing organic substituents and the like. Further, thickening agents and/or metal soaps in grease-forming proportions or in amounts insufficient to form grease may be utilized in combination with the addition agents of this invention.

While the character of the invention has been described in detail and numerous examples of the compounds given, this has been done by way of illustration only and with the intention that no limitation should be imposed upon the invention thereby. It will be apparent to those skilled in the art that numerous modifications and variations of the illustrative examples may be effected in the practice of the invention which is of the scope of the claims appended hereto.

We claim:

1. A composition comprising a hydrocarbon oil containing a small amount of a salt of a substituted acid of boron containing an organic substituent, said small amount being at least about 0.05% by weight.

2. A composition comprising a hydrocarbon oil containing from about 0.1% to about 2% by weight of a metal salt of a substituted acid of boron containing an organic substituent.

3. A composition comprising a hydrocarbon oil containing from about 0.1% to about 2% by weight of a polyvalent metal salt of a substituted acid of boron containing an organic substituent.
- 5 4. A composition comprising a hydrocarbon oil containing from about 0.1% to about 2% by weight of an ammonium salt of a substituted acid of boron containing an organic substituent.
- 10 5. A composition comprising a hydrocarbon oil containing from about 0.1% to about 2% by weight of an amine salt of a substituted acid of boron containing an organic substituent.
- 15 6. A composition comprising a hydrocarbon oil and from about 0.1% to about 2% by weight of a compound containing the group—  
(A) (X) (B) (R)
- in which A is a metal, X is selected from the group consisting of oxygen, sulfur and selenium, 20 B is boron, and R is an organic radical.
7. A composition as defined in claim 6 in which A is a polyvalent metal.
8. A composition comprising a hydrocarbon oil and at least about 0.05% by weight of a salt of an acid ester of an acid of boron.
- 25 9. A composition comprising a hydrocarbon oil and at least about 0.05% by weight of a metal salt of an acid ester of an acid of boron.
10. A composition comprising a hydrocarbon oil and at least about 0.05% by weight of a polyvalent metal salt of an acid ester of an acid of boron.
- 30 35 11. A composition comprising a hydrocarbon oil and from about 0.1% to about 2% by weight of a salt of an oxyacid of boron containing an organic substituent.
12. A composition comprising a hydrocarbon oil and from about 0.1% to about 2% by weight of a salt of a sulfur-containing acid of boron having an organic substituent.
- 40 45 13. A composition comprising a hydrocarbon oil and from about 0.1% to about 2% by weight of a salt of an organo-boronic acid.
14. A composition comprising a hydrocarbon oil and from about 0.1% to about 2% by weight of a salt of an organo-borinic acid.
- 50 15. A composition comprising a hydrocarbon oil and from about 0.1% to about 2% by weight of a salt of an orthoboric acid containing an organic substituent.
16. A composition comprising a hydrocarbon oil and from about 0.1% to about 2% by weight of a salt of a dibasic orthoboric acid containing an organic substituent.
- 55 17. A composition comprising a hydrocarbon oil and from about 0.1% to about 2% by weight of a salt of a monobasic orthoboric acid containing an organic substituent.
18. A compounded lubricant comprising a lubricating oil subject to deterioration at elevated temperatures and a salt of an acid of boron containing an organic substituent, said salt being present in an amount sufficient substantially to inhibit said deterioration.
- 60 65 19. A compounded lubricant comprising a lubricating oil subject to deterioration at elevated temperatures and a metal salt of an acid of boron containing an organic substituent, said salt being present in an amount sufficient substantially to inhibit said deterioration.
- 70 75 20. A compounded lubricant comprising a lubricating oil subject to deterioration at elevated temperatures and a polyvalent metal salt of an acid of boron containing an organic substituent, said salt being present in an amount

sufficient substantially to inhibit said deterioration.

21. A compounded lubricant comprising a hydrocarbon oil with the properties of such composition affecting its use as a lubricant improved by incorporating therein at least 0.05% by weight based on the oil of a salt of an acid of boron containing an organic substituent.

22. A compounded lubricant as defined in claim 21, in which said salt is a polyvalent metal salt.

23. A compounded lubricant comprising a hydrocarbon oil with the properties of such composition affecting its use as a lubricant improved by incorporating therein at least 0.05% by weight based on the oil of a salt of an organic acid ester of an acid of boron.

24. An addition agent capable of inhibiting deterioration of lubricating oils which comprises a concentrated solution in oil of a salt of

an organic substituted boron compound, said concentrated solution containing more than 2% by weight based on the oil of said salt and being capable of dilution with mineral lubricating oil to form a homogeneous mixture containing from approximately 0.05% to 2% by weight of said salt.

25. An addition agent capable of inhibiting deterioration of lubricating oils which comprises a concentrated solution in oil of a polyvalent metal salt of an acid of boron containing an organic substituent, said concentrated solution containing more than 2% by weight based on the oil of said salt and being capable of dilution with mineral lubricating oil to form a homogeneous mixture containing from approximately 0.05% to 2% by weight of said salt.

JAMES O. CLAYTON.  
BRUCE B. FARRINGTON.